

I. S. JOSEPH.

METHOD OF RECOVERING THE INGREDIENTS FROM WASTE ROOFING, &c.  
APPLICATION FILED NOV. 1, 1916.

1,253,386.

Patented Jan. 15, 1918.

*Fig. 1.*



*Fig. 2.*



*Fig. 3.*



Irwin S. Joseph,

By *Byron, Townsend & Dickstein,*

Attorneys.

# UNITED STATES PATENT OFFICE.

IRWIN S. JOSEPH, OF RAHWAY, NEW JERSEY.

## METHOD OF RECOVERING THE INGREDIENTS FROM WASTE ROOFING, &c.

1,253,386.

Specification of Letters Patent.

Patented Jan. 15, 1918.

Application filed November 1, 1916. Serial No. 129,015.

*To all whom it may concern:*

Be it known that I, IRWIN S. JOSEPH, a citizen of the United States, residing at Rahway, in the county of Union and State 5 of New Jersey, have invented certain new and useful Improvements in Methods of Recovering the Ingredients from Waste Roofing, &c., of which the following is a specification.

10 This invention relates to a method for reclaiming the ingredients from scraps or pieces of plastic strip-roofing or the like, such as is well known in the roofing-trade today, having a bituminous binder.

15 One type, for instance, of roofing of this character comprises a layer of felt or similar fabric impregnated with asphalt and having a granular superficial layer of hard mineral substance, such as slate. In the cutting and other operations about the factories where such roofing material is made, a large quantity of the material goes to waste as scraps, notwithstanding the fact that the ingredients thereof, if recovered, would pro-

20 vide substantial amounts of re-usable material. On account of the manner in which this roofing is made, it is practically impossible to effectively separate the ingredients thereof by any so-called "dry" process.

25 According to my invention as hereinafter described, the several ingredients are recovered from the waste material, by a process so simple and inexpensive as to render the same highly practicable, which, of course, is 30 the feature of primary consideration in operations of this nature.

Briefly, the invention comprises the introduction of the waste pieces of roofing into a liquid separating-medium immiscible with 35 the bituminous material, of greater specific gravity and maintained at a temperature sufficiently high to effect melting of the bituminous material and thereby disengage the fabric and stone-particles. The bituminous material may be withdrawn from the 40 top of the separating-medium, while the other ingredients can be removed from the lower portion of the medium.

45 The invention will be better understood by reference to the accompanying drawing, wherein—

Figure 1 is a plan view of a piece of roof-

ing-strip made from materials which the present process is intended to recover;

Fig. 2 is a sectional view of the same; and 55

Fig. 3 illustrates a suitable apparatus in which the process may be carried out.

As illustrated in Fig. 1 the roofing-material may comprise a lower layer 1 of felt or other fabric impregnated with bituminous 60 material, such as asphalt, and a surface coat 3 of granular slate, slag or rock, rolled in the well known manner upon the impregnated fabric, or into its additional asphalt covering 2 which is sometimes applied. 65

In carrying out the process of the present invention, the scraps of such roofing-material are introduced into a vessel 4, having a removable cover 4', and containing preferably a saturated solution 5 of the salt, such 70 as sodium chlorid, sufficient heat being applied by the introduction of steam through the perforated coil 6 to effect melting of the asphalt contained in the pieces and consequent release of the felt and hard mineral 75 substance. The asphalt or other bituminous material thereupon immediately rises to the surface of the separating-medium 5, as indicated by the numeral 7, while the heavier ingredients 7' consisting, for instance, of slate 80 and felt, gravitate to the bottom of the vessel, from which they may be withdrawn through the valved outlet 8. The asphalt may be conveniently withdrawn through the valved outlet 9. Fresh salt solution may be 85 supplied as needed through the inlet-pipe 10.

If desired the withdrawn asphalt may be further treated for refinement, or it may be utilized in substantially its recovered condition in the manufacture of new roofing-material. The heavy portions 7', withdrawn 90 from the vessel 4 through the outlet 8, are subjected to a further treatment for the separation of the mineral substance from the felt. Such separation may be effected 95 by flotation, as indicated in the drawing, or it may be accomplished by a vibrated belt or other known contrivance.

In this manner, substantially all of the ingredients may be recovered and utilized in 100 the preparation of fresh roofing, this not having been hitherto attempted because of the necessary trouble and expense incident to the processes heretofore suggested.

I claim:—

The method of recovering the ingredients from waste roofing of the asphalt-felt-stone variety, comprising introducing the waste 5 roofing into a liquid separating-medium immiscible with the asphalt, of greater specific gravity and maintained at a temperature sufficiently high to effect melting of the asphalt and disengagement of the felt and

stone, separately recovering the asphalt, felt 10 and stone from the solution, and thereafter mechanically separating the felt and stone.

In testimony whereof I affix my signature in presence of two witnesses.

IRWIN S. JOSEPH.

Witnesses:

A. J. SCHWINDINGER,  
T. M. VAN DERVEER.